

A. J. BOYNTON & A. E. SANDS.

PROCESS OF SINTERING.

APPLICATION FILED AUG. 3, 1917.

1,245,183.

Patented Nov. 6, 1917.

2 SHEETS—SHEET 1.

FIG. 3



FIG. 2



FIG. 1



WITNESSES

R. Shatto  
W. T. Holman

INVENTOR

A. J. Boynton  
A. E. Sands  
D. Allgaier  
Their Attorney

**A. J. BOYNTON & A. E. SANDS.**  
**PROCESS OF SINTERING.**  
**APPLICATION FILED AUG. 3, 1917.**

**1,245,183.**

Patented Nov. 6, 1917.

2 SHEETS—SHEET 2.



**WITNESSES**

R. D. Latta  
W. T. Holman

## INVENTOR

A. J. Boynton  
A. E. Saude  
" of Alabama  
their Attorney

# UNITED STATES PATENT OFFICE.

ARTHUR J. BOYNTON, OF LORAIN, AND ALBERT E. SANDS, OF AKRON, OHIO.

## PROCESS OF SINTERING.

1,245,183.

Specification of Letters Patent.

Patented Nov. 6, 1917.

Application filed August 3, 1917. Serial No. 184,296.

*To all whom it may concern:*

Be it known that we, ARTHUR J. BOYNTON and ALBERT E. SANDS, citizens of the United States, and residents, respectively, of Lorain, in the county of Lorain and State of Ohio, and Akron, in the county of Summit and State of Ohio, have invented a new and useful Process of Sintering, of which the following is a specification.

10 Our invention relates to sintering blast furnace flue dust, iron ores, and similar finely divided materials which are combustible or to which a combustible is added in preparation for sintering. While not necessarily limited to such apparatus, our improved process is particularly adapted for use with sintering apparatus embodying a sintering pan having a porous hearth formed of refractory material, and having 20 means for causing a current of air to pass through a body of the sintering material positioned in such pan in quantities sufficient to support combustion and cause the materials to sinter.

25 In the sintering processes heretofore used in connection with apparatus such as that shown, a quantity of flue dust or other combustible material in a finely divided state is placed in the sintering pan. Usually, and 30 preferably, the grate bars forming the perforated bottom of the sintering pan are covered with a layer of crushed limestone or similar refractory material to form a porous hearth within the sintering pan upon which 35 the material being sintered is supported.

After the upper surface of such body of flue dust in the sintering pan is leveled, a gas burning igniter is wheeled or otherwise moved into position above the material, or 40 above a portion of the material, in the sintering pan. An exhaust fan, which is connected to the bottom of the sintering pan in any suitable manner, is then started in operation and the gas burning igniter is 45 lighted.

The igniter then fires the upper surface of the material within the pan that is covered by the igniter, the exhaust fan withdrawing the products of combustion from 50 the pan and causing a current of air to pass through the material in the pan in quantities sufficient to support combustion and cause the formation of sinter. After the upper surface of the material within the 55 sintering pan is thoroughly ignited and the sintering operation is started, the igniter

is moved away from above the pan. The exhaust fan continues to withdraw the products of combustion from the pan and by suction, draws sufficient air into or 60 through the body of materials in the sintering pan to gradually propagate the sintering operation throughout the mass or body of material within the sintering pan.

The sintering of flue dust and fine ores 65 is only made possible by reason of the carbon or a similar combustible in the material being sintered, carbonaceous material being added to the iron ore when such ore is the material to be sintered.

70 The amount of carbon in the material to be sintered, unless carefully regulated so as to be but slightly in excess of the amount required to support combustion, causes a very intense heat. Such high temperatures 75 necessitate a long time to be taken in cooling the sinter, while it is a general rule that the greater the amount of carbon in the material the larger will be the amount of cinder formed in the sintering operation. 80

It is not practicable to maintain the carbon content of the materials within the close range between that necessary to support combustion and that required in order to prevent a large increase in the temperature of the sintered material and the formation of large quantities of cinder that results from an excess amount of carbon, without such frequent and careful sampling and analyses as will make the cost prohibitive. 85

It, heretofore, has been necessary to consume a considerable part of the time in cooling the sintered mass after the sintering operation is completed from the high temperature at which it is completed and there- 90 by delay the sintering operations, while the molten cinder formed in the sintering operation clogs and chokes up the voids in the porous hearth and seriously interferes with the completion of the sintering operation, 95 in the last stages of each sintering operation. It frequently occurs that owing to the shutting off of the air supply in this way, as much time is required to sinter the last ten per cent. of the material in the sintering pan as is necessary to sinter the first 100 ninety per cent.

One object of our invention is the provision of a novel method of sintering whereby the sintering operation is facilitated, the 110 time required in cooling the sinter is reduced, and whereby the sinter is rapidly

and more uniformly cooled and the hardness and porosity are equalized and made uniform throughout the sintered mass.

Another object of our invention is to provide an improved method of sintering whereby wide variations in the carbon content of the material being sintered are rendered negligible without interference with the sintering operation or lessening of the quality of the sinter.

A further object of our invention is to provide an improved process of sintering having a novel series of steps whereby the sintering operation is facilitated and whereby the character of the sinter as to porosity and hardness is rendered much more uniform.

A still further object of this invention is to provide a novel process of sintering whereby the molten cinder formed in the sintering operation is drained off as formed from the body of the materials being sintered, and choking of the passages for the air and products of combustion during the sintering operation, is avoided and prevented.

A further object of the invention is to provide an improved process of sintering having a novel series of steps whereby interference with and delays in the completion of the sintering operation by the formation of molten cinder during the sintering operation, are lessened and overcome.

Referring now to the drawings, forming part of this specification, Figure 1 is a diagrammatic plan showing one embodiment of sintering apparatus which is constructed and arranged and adapted for use in carrying out our improved process.

Fig. 2 is a diagrammatic side elevation of the apparatus shown in Fig. 1.

Fig. 3 is a diagrammatic end elevation of the apparatus shown in Figs. 1 and 2.

Fig. 4 is a sectional end elevation showing details in the construction and arrangement of the tilting sintering pan forming part of the apparatus shown in the preceding figures of the drawings.

Fig. 5 is a sectional plan showing a detail in the construction of the connection between the stationary exhaust conduits and tilting sintering pan of the apparatus shown in the preceding figures of the drawings.

In the accompanying drawings, the numeral 2 designates a sintering pan which is arranged to tilt or rock about a horizontal axis, opposite ends of this pin being provided with hollow trunnions 3, 3, by which the pan is rotatably mounted in suitable trunnion bearings.

The pan 2 has a bottom 5, sides 6, 6, and integrally formed ends 7, the hollow trunnions 3, 3, opening into the pan through the end walls of the pan. At an intermediate point in the height of the side walls of the

pan is a series of perforated grate bars 8, these grate bars being fastened in place within the pan 2 in any desired manner, and loosely positioned on top of the grate bars is a porous hearth 9 formed of a thin layer of crushed limestone or similar refractory material.

The outer ends of the hollow trunnions 3 are connected to one end of pipes which form conduits 10, 10, for leading the gaseous products of combustion from beneath the grate bars 8 in the pan 2 into the exhaust blower or fan 11 to which one end of each of the pipes 10, 10, are connected. The exhaust blower or fan 11 which, as shown, has two inlets, has a single discharge outlet which is connected by a branch pipe 12 to the lower end of a stack 13, the stack being of sufficient height to carry off the products of combustion discharged thereinto by the exhaust fan.

The tilting sintering pan 2 is elevated above the ground level and is arranged to be rotated on the trunnion bearings through an arc of at least 180 degrees, in order that it can be positioned horizontally to receive successive quantities of material to be sintered and to enable the igniter 14 to be moved into and out of position above the pan, and also to permit of the pan being tilted at an angle to the horizontal after the sintering operation is commenced and to be inverted so as to discharge the sinter from the pan 2 into a car 15 positioned on the track 16 located in line with and below the elevated sintering pan 2.

A suitable turning mechanism will be provided for the tilting pan as well as means for tempering and mixing the finely divided materials to be sintered, and means for delivering or discharging the materials into the sintering pan.

In the operation of our improved process the flue dust or other material to be sintered will be placed in an overhead bin or bunker. Weighed quantities of the material will be withdrawn from the bunker and placed in a rotary mixer. Sufficient water will be added to the weighed materials, either before or after being placed in the mixer, and the materials will be thoroughly mixed and tempered.

The materials are then removed from the mixer and placed in the sintering pan, preferably a chute being employed to deliver the materials into the pan by gravity. The materials in the pan are then leveled, after which the gas burning igniter is moved into position above the pan of materials to be sintered.

The exhaust fan 11 is then started and the igniter 14 is lighted. The fan creates suction within the pan 2 and draws air and the products of combustion through the body of materials and the porous hearth 9 in the

pan, and discharges the gaseous products of combustion into the stack 13. After the upper surface of the materials in the sintering pan 2 is thoroughly fired or ignited, the 5 igniter is removed from above the sintering pan and the sintering operation is allowed to progress. After the sintering operation has extended over the upper surface of the material in the sintering pan and the 10 material is sintered to a sufficient extent to form a crust on the outer surface of the material in the pan, the pan is tipped or tilted until the upper surface of the materials in the pan is at an angle somewhat less than a 15 right angle to the horizontal. The sintering operation is then allowed to propagate throughout the mass until the entire body of materials within the pan is formed into sinter.

20 As the pan 2 is tilted at an angle to the horizontal during the major portion of the time required in sintering, any molten cinder formed during the sintering operation will trickle downwardly at an angle to the 25 horizontal or approximately horizontal path or direction of travel of the column of air used in supporting combustion, and when sufficient quantities are formed, will flow out of the pan. The flow of molten cinder 30 will be furthered by punching a series of holes in the sintered crust on the mass of sintering material in the pan 2 adjacent to what forms the lower edge of the tilted pan 2 during the sintering operation. The porous 35 hearth 9 in the sintering pan, extending at an angle to the horizontal, during the time molten cinder is formed in the materials being sintered, freezing of the cinder in the voids in the porous hearth and in the 40 adjacent surfaces of the materials being sintered is prevented, and clogging of the voids by the cinder and the resulting retardation or shutting off of the air supply due to 45 choking up of the voids in the porous hearth as occurs in the prior processes, is avoided and overcome.

As the latter part of each sintering operation is not retarded by clogging of the porous hearth, the material in the pan is uniformly sintered throughout the thickness of the mass, and spots or patches of unsintered materials are not found on the bottom surface of the mass, as in the case of the processes heretofore known. The air supply 50 not being lessened by clogging of the porous hearth by cinder freezing thereon, currents of air are freely drawn through the sintered mass which is porous after the completion of the sintering operation so as 55 to hasten cooling of the mass and prevent the long delays in the completion of the sintering operation heretofore caused in cooling the sinter.

After the mass of sinter in the pan 2 60 has been cooled to the desired extent, the

pan is further tilted so as to be inverted and the sinter is thereby discharged into the car 15 positioned on the track 16 beneath the sintering pan. The sinter having been cooled to the desired extent, the last sintered portions of the mass will not break up into pieces smaller than is desired in the use to which the sinter is put.

The above described operations are then carried out with successive quantities of sintering material.

The advantages of our improved process, which will be appreciated by those skilled in the art arise from the use of a process wherein the cinder is drawn off as formed 70 from the materials being sintered, and is removed from the sintering mass so as to prevent shutting off of the air supply and avoid forming sinter which is not uniform in hardness and porosity. By removing 75 the cinder as formed from the sintering mass, the use of materials have large variations in the amount of carbon or other combustible material is made possible without the necessity of frequent and correspondingly costly sampling and analyses of the 80 materials.

Modifications in the steps of our improved process may be made without departing from the spirit of the invention as defined 95 in the claims, and various types of apparatus may be employed in carrying out our invention.

We claim:

1. The process of sintering flue dust and 100 similar combustible materials which consists in igniting a body of the material, forcing air through the ignited mass to support combustion and propagate the sintering operation throughout the mass, and tilting the ignited mass to drain the molten cinder as formed therein.

2. The process of sintering flue dust and 105 similar combustible materials which consists in supporting a bed of the materials 110 on a porous hearth, igniting one face of the so-formed bed, forcing sufficient air into the bed to promote combustion and propagate the sintering operation throughout the bed, and tilting the bed during the sintering operation to drain molten cinder as formed 115 therein.

3. The process of sintering which consists 120 in supporting a bed of the material to be sintered on a porous hearth, igniting the upper face of the material, forcing air downwardly through the material to promote combustion and propagate the sintering thereof, and tilting the bed of material during the sintering operation to drain molten 125 cinder formed therein during the sintering operation.

4. The process of sintering which consists 130 in forming a bed of combustible sintering material, igniting one horizontal face of

- said bed, passing air through the ignited bed in a direction at right angles to the ignited face of the bed to support combustion and form a crust on said ignited face, 5 and then tilting the bed and thereby drawing off molten cinder downwardly in a direction substantially parallel to the plane of the ignited face of said bed of material in completing the sintering operation.
- 10 5. The process of sintering which consists in forming a bed of combustible sintering material, igniting the upper horizontal face of said bed, passing air through the ignited

bed in a direction at right angles to the ignited face of the bed to support combustion and form a crust on said ignited face, 15 and then tilting the bed and thereby drawing off molten cinder downwardly in a direction substantially parallel to the plane of the ignited face of said bed of material 20 in completing the sintering operation.

In testimony whereof we have hereunto set our hands.

ARTHUR J. BOYNTON.  
ALBERT E. SANDS.